

# UNITED STATES PATENT OFFICE.

RENÉ BOHN, OSCAR BALLY, AND HUGO WOLFF, OF MANNHEIM, GERMANY, ASSIGNEES  
TO BADISCHE ANILIN & SODA FABRIK, OF LUDWIGSHAFEN-ON-THE-RHINE, GERMANY, A CORPORATION.

## TANNING.

1,281,494.

Specification of Letters Patent. Patented Oct. 15, 1918.

No Drawing.

Application filed December 30, 1916. Serial No. 139,872.

To all whom it may concern:

Be it known that we, RENÉ BOHN, OSCAR BALLY, and HUGO WOLFF, the first and second citizens of the Swiss Republic and the 5 third citizen of the German Empire, residing at Mannheim, Germany, have invented new and useful Improvements in Tanning, of which the following is a specification.

As is known the natural tanning materials hitherto employed all possess an amorphous character.

Now we have made the discovery that we can transform hides into a valuable leather of good properties by treating them with an 15 aqueous solution of sulfonated aromatic hydrocarbons containing a system of at least three condensed nuclei, which sulfonated products generally represent substances of a crystalline character. As instances of hydrocarbons of the aforesaid kind we mention anthracene, phenanthrene, fluorene and the like, or derivatives thereof, such as halogen substitution products of the said hydrocarbons. The said sulfonated products can 20 be employed either alone or in the form of mixtures of several sulfonic acids of the same hydrocarbon or of different hydrocarbons and an addition can be made of other tanning materials or other suitable bodies. 25 Besides, the tanning process can be carried out in the ordinary manner. Suitable mixtures of sulfonated hydrocarbons can be produced by treating, for instance, anthracene with a sulfonating agent so as to give rise 30 to a mixture of anthracene disulfonic acids, or, by sulfonating crude anthracene, containing phenanthrene, fluorene and like hydrocarbons, so as to produce a mixture of sulfonic acids of the said hydrocarbons. The 35 sulfonic acids can be directly employed in the free state or their salts, in particular their alkali salts, can be used with an addition of an acid.

For the purpose of further illustrating the 45 invention we give the following examples, but the invention is not confined to these examples. The parts are by weight.

### Example 1.

50 Dissolve, at ordinary temperature, 50 parts of a mixture of the sodium salts of anthracene, 1.5 and 1.8-disulfonic acids (prepared by sulfonating anthracene of about 80 per cent. purity and purifying, if 55 desired, by means of the calcium salts) in

1000 parts of water, acidify the solution by adding 50 parts of dilute sulfuric acid of 10%, introduce into this solution the hides which are deprived of lime by a treatment with bisulfite solution and treat until the 60 hides are thoroughly tanned. The leather is then washed and fatted in the usual way; it is of a brown color with brown cut and possesses good strength.

65

### Example 2.

Dissolve 40 parts of dichlor-anthracene-disulfonic acid in 1000 parts of hot water, acidify by adding 100 parts of dilute sulfuric acid of 10% and allow to cool. Then 70 introduce the hides which are deprived of lime by treatment with bisulfite solution and treat until the hides are thoroughly tanned. The leather is finished as usual; it has a 75 dull yellow color with a light reddish yellow cut and possesses a strong fiber condition.

In an analogous manner, hides can be tanned with solutions of other sulfonic acids of anthracene, such as anthracene-1-sulfonic acid sodium salt, anthracene-2-sulfonic acid, anthracene-1.5- or -1.8- or -2.6- or -2.7-disulfonic acid sodium salts, or 1.4-dichlor-anthracene-sulfonic acid sodium salt and the like.

### Example 3.

70 parts of the mixture of the potassium salts of phenanthrene 2- and 3-sulfonic acids, such as is obtainable as described in *Annalen der Chemie* vol. 321, p. 251 or *Berichte der Deutschen Chemischen Gesellschaft*, vol. 34, p. 4004, are dissolved at the ordinary temperature in 1000 parts of water and added with 70 parts of sulfuric acid of 10%. Then introduce the hide treated with bisulfite solution and treat until it is thoroughly tanned. The leather is finished as usual. It is a slightly swelled leather of a brown 95 color turning to white in the interior.

The phenanthrene-2 and 3-sulfonic acid 100 can be replaced by the sodium salts of the mixed sulfonic acids obtained by sulfonating crude phenanthrene of say 84 per cent. purity. A brown leather with a light brown cut is thereby obtained possessing a soft condition and good grain.

### Example 4.

70 parts of the mixture of fluorene sulfonic acid sodium salts, obtained by sul-

110

fonating fluorene with sulfuric acid of 66%, are dissolved in 1000 parts of warm water and acidified with 70 parts of sulfuric acid of 16%. When cold, the hides, treated with 5 bisulfite solution, are introduced and treated until they are thoroughly tanned. Then the leather is washed and fatted in the ordinary manner. It is a slightly swelled leather with soft grain and a yellowish-white color. In 10 an analogous manner the easily soluble disulfonic acids of fluorene (see *Annalen der Chemie* vol. 390, p. 217) can be employed. They yield a soft yellowish leather.

We claim:

- 15 1. The process of tanning hides which comprises treating hides with a bath containing a sulfonated aromatic hydrocarbon which consists of a system of at least three condensed nuclei.
- 20 2. The process of tanning hides which comprises treating hides with a bath containing the sulfonic acids of the hydrocarbons contained in crude anthracene.
- 25 3. The process of tanning hides which comprises treating hides with a bath containing an anthracene sulfonic acid.
4. The process of tanning hides which comprises depriving hides of lime and then treating them with a bath containing a sul-

fonated aromatic hydrocarbon which consists of a system of at least three condensed nuclei. 30

5. The process of tanning hides which comprises depriving hides of lime and then treating them with a bath containing an anthracene sulfonic acid. 35

6. The process of tanning hides which comprises depriving hides of lime and swelling them and then treating them with a bath containing an anthracene sulfonic acid. 40

7. The process of tanning hides which comprises treating hides with a bath containing an anthracene sulfonic acid salt and an acid.

8. As a new article of manufacture a 45 leather containing as a tanning constituent a sulfonated aromatic hydrocarbon which consists of a system of at least three condensed nuclei.

9. As a new article of manufacture a 50 leather containing as a tanning constituent a sulfonated anthracene derivative.

In testimony whereof we have hereunto set our hands.

RENÉ BOHN.  
OSCAR BALLY.  
HUGO WOLFF.